

1

2,739,106

## METHOD OF ELECTROPLATING COPPER-LEAD ALLOY

Wilbur G. Hespenheide and Charles L. Faust, Columbus, Ohio, assignors, by mesne assignments, to American Brake Shoe Company, New York, N. Y., a corporation of Delaware

No Drawing. Application June 25, 1952,  
Serial No. 295,543

8 Claims. (Cl. 204—23)

This invention relates to electrodeposited copper-lead alloys and methods for the electrodeposition thereof. In particular, it relates to electrodepositing liners of copper-lead alloys on bearing shells of steel or other metal.

It is well known in the metallurgical field that copper-lead bearing liners have superior properties for use in heavy-duty service for industrial engines and machinery. According to present-day practice in this field, copper-lead alloys are first prepared by melting copper and lead together and are then cast in molten form onto the inside surface of cylinder of steel or other metal. The copper-lead alloy may also be cast onto a flat strip, of the proper thickness, which is subsequently cut to the desired lengths and formed into bearing half-shells.

Due to the fact that the lead and copper are, for all practical purposes, insoluble in each other in the solid and liquid state, the copper-lead alloy bearing liners formed by these methods consist of a lace work or dendritic structure of copper, surrounded by metallic lead. Thus, during solidification of a mechanical mixture of copper and lead, the copper crystallizes in a dendritic structure, and the lead then solidifies in the region between these dentrites. Such separation between the two constituents might be advantageous, since the lead phase has a lubricating property which is highly desirable in bearing performance. However, the segregation of lead also causes a serious disadvantage, since there is a pronounced tendency for the lead to separate out in a continuous layer at the interface between the metal backing element and the copper-lead alloy bearing layer. This interfacial layer of lead presents a zone of mechanical weakness, and consequently the performance of the bearing is not as satisfactory as it would be if such lead zone were not present between the metal backing member and the copper-lead alloy bearing liner.

Of course, enhancement of bearing performance is directly related to the extent and uniformity with which lead is dispersed in the copper matrix. Thus, inherent lubricating effects are increased, noise is eliminated to a greater extent, and the bearing is easier to machine. Prior attempts to prepare suitable copper-lead bearings by casting methods in which there is a satisfactory quantity, dispersion, concentration, and distribution of lead in copper have been retarded and made difficult by, among other things, differences in the melting point of copper and lead; separation of lead upon cooling rather than on alloying thereof with copper; and the difference in specific gravity between the two metals.

For many years the bearing industry has sought ways to produce a copper-lead alloy bearing liner without the inherent disadvantages that result from preparing the alloy by melting and casting techniques. One of the methods proposed has been the simultaneous electrodeposition of copper and lead. Numerous suggestions have been made for electrodepositing copper-lead alloys, but none has produced an alloy plate having the proper com-

2

position and, at the same time, possessing the required physical properties for a bearing liner.

The prior-art copper-lead alloy plating developments have produced copper-lead electrodeposits that were either extremely brittle or wholly unsuitable for bearing liners due to the fact that the codeposited copper and lead were noncoherent and appeared as a powdery sponge-like metal. Further, the codeposits of copper and lead reported in the technical literature are extremely hard, not being amenable to customary metallurgical heat treatments, and have, therefore, resisted annealing to the lesser hardness which is desirable for bearing metal.

It has been proposed, as a specific example, to codeposit copper and lead from a bath containing copper hydroxide and lead acetate. This deposit, however, is characterized by many hair line cracks forming an irregular network extending from the surface of the deposit to the face of the backing metal. Further, the deposit is laminar in form, layers of lead occurring between adjacent copper layers and also there is an irregular dispersion of lead in the copper matrix. As a consequence, the deposit is brittle and incapable of practical use, and in an attempt to properly and satisfactorily relate the copper and lead phases, a special annealing technique is employed. However, a satisfactory softness can be attained only by annealing at temperatures above the melting point of lead for a prolonged period. This heat treatment causes the lead to sweat out forming an interfacial layer of lead as in casting techniques and also large aggregations of lead on the surface of the deposit. In addition, gross copper recrystallization grains are produced, and it will be seen that while the desired softness is attained, a much weakened structure is produced. This prior method for producing copper-lead bearing linings by co-deposition on a suitable backing is typical of what has heretofore been accomplished in the art.

It is well known in the art of alloy plating that there is no obvious equivalency between the methods for electrodepositing one or more pure metals directly and methods for electrodepositing alloys of these metals. In other words, the nature of the art is such that there is no suggestion or provision which makes it possible to take a satisfactory electrodeposition bath for copper on one hand and for lead on the other, mix them together, and thus obtain a suitable copper-lead alloy plating solution which will thereby give an alloy having predetermined properties selected for a given usage.

There are, of course, known methods of alloy plating by which alloys of two or more metals can be formed. These are especially useful when other methods, such as melting and casting, are unsuccessful. Again, however, that same knowledge does not teach the procedure by which known plating methods can be combined to immediately produce the desired results. All this is clearly shown by the known methods of electrodepositing copper and lead as pure metals. For example, copper can be deposited in good form for many uses from a copper fluoborate solution. Yet, when copper fluoborate and lead fluoborate are in the same solution, either a powdery, spongy codeposit of lead and copper, or a very hard, extremely brittle codeposit of copper and lead is obtained, when alloys comprising over 25 per cent copper are sought. Neither of these codeposits is suitable for a bearing metal.

Likewise, it is known that copper can be deposited from a cyanide solution which contains free alkali as well as free cyanide. Lead has been deposited from a solution of lead oxide in an alkaline tartrate solution. Yet when the alkaline cyanide-copper solution and the alkaline tartrate-lead solution are mixed, the resulting solution

will not produce the satisfactory codeposition of copper and lead which is required for bearings.

A desirable and usable copper-lead alloy deposit might be expected if the teachings of alloy plating were directly transferable from one pair of metals to another. The technical literature shows that an alkaline silver cyanide-lead tartrate solution can electrodeposit a very satisfactory bearing alloy of high-silver and low-lead composition. Yet attempts to electrodeposit a suitable high-copper low-lead alloy from a comparable solution is totally without success.

It is recognized that codeposits of copper and lead can be obtained in a dense metallic form. However, this type of alloy is too brittle and too hard to be used as a bearing material. Furthermore, the alloy cannot be softened by customary heat treatments to produce a product having a suitable ductility and hardness.

In accordance with the present invention, it has now been found that suitable copper-lead alloys can be electrodeposited, and it has also been discovered that by heat-treating such alloys the same can be softened for use as a bearing material on a steel or equivalent backing member. Further, by the same technique, to be described hereinafter, the copper-lead alloy plate can be electrodeposited on other bearing backing materials to produce a bearing-alloy liner.

The present process is based on a combination of copper and lead salts which has not heretofore been known or ever shown to be useful in electrodepositing alloys. For example, we have found that a combination of copper-cyanide and lead pyrophosphate produces a stable solution in water, and that this solution will give copper-lead alloy codeposits which can be subsequently heat-treated to produce satisfactory bearing liners.

It is, therefore, an object of this invention to electrodeposit copper-lead alloys by a novel process.

It is another object of this invention to effectively electrodeposit copper-lead alloys on a metal backing material and subsequently treat the alloys to provide a satisfactory bearing.

It is a further object of this invention to avoid in copper-alloy electrodeposits having a metastable solid solution of lead in copper harmful segregations of lead that render such deposits detrimental for use as a satisfactory bearing material.

Yet another object of this invention is to produce high-copper, low-lead alloy electroplates.

Further objects should be apparent from what has heretofore been discussed and outlined, and other objects are also embodied in the description to follow as will be appreciated by those who are skilled in the art.

Desired alloy compositions for most general bearing use are in the range of from 5 to 20% lead, balance copper. It has been found, in accordance with the present invention, that copper-lead alloys containing from 5 to 95% lead can be electrodeposited from cyanide-pyrophosphate baths, and that these baths are stable during long periods of continuous use. The desired high-copper, low-lead alloys are obtained in a form which can be suitably heat-treated, as will hereinafter be described.

The alloy electroplates in this composition range are, according to X-ray examination, solid solutions of lead in copper, since X-ray analysis in the present instance shows only a copper phase with a strained lattice. This solid solution is totally unpredicted by the usual thermal diagrams of copper-lead alloys, since the solubility of lead in copper certainly lies well below 1/2% yet it is the result of the infinitely fine process of atom-by-atom co-deposition of copper and lead. The resulting solid solution is very stable during ordinary low-temperature heat treatment, and in view of the fact that this absolute condition of solubility is, thermally speaking, not a normal one, such solutions occurring as the result of present practice will be referred to as "metastable."

The plating bath for the copper-lead alloy electro-

deposition comprises a water solution containing copper-cyanide and lead-pyrophosphate complexes. Lead pyrophosphate is the only known inorganic salt of lead which is appreciably soluble in the pH range of 6 to 10. Since lead forms no cyanide complex, it is necessary to have lead in a complex with so little ionization that there are substantially as few free lead ions in the solution as there are copper ions in the solution of copper-cyanide. Lead-pyrophosphate forms such a complex, and thus has been found to be highly desirable for codepositing copper and lead in an alloy form that is suitable for bearing performance. Since suppressed copper forms no pyrophosphate complex when cyanide is present, an excellent copper-lead alloy electrodepositing bath is formed by having copper-cyanide and lead pyrophosphate complexes present in the same solution.

The lead pyrophosphate complex is formed by addition to water of an alkali pyrophosphate salt and a soluble lead salt which will ionize to form plumbous lead. Copper-cyanide is added to the bath, and an additional amount of an alkali metal cyanide is added to suppress the copper. It may also be desirable to add an alkali metal dihydrogen orthophosphate for the purpose of buffering against changes in pH.

The amount of the bath components are dependent on the composition of alloy desired, and pH of the solution, and other factors. In general, an increase in the alkali metal cyanide concentration will result in a decrease in the copper content of the plate. As has been heretofore stated, the pH of the bath must be maintained within the range of about 6 to 10, in order to keep the lead pyrophosphate from precipitating out of solution. The temperature of the bath during electrodeposition should range from about 110° to 170° F. An increase in bath temperature will result in an increase in the copper content of the alloy deposited.

In the electrodeposition of the alloy the metal surface to be coated is made the cathode, the anodes preferably being made from an alloy having approximately the same composition as that desired in the bearing liners. It is also possible to use pure copper anodes, and in this case periodic additions of suitable salts are necessary to maintain the desired concentration of lead in the bath. As an alternative arrangement, there may be provided individual anodes of lead and copper using a dual anode circuit. The areas of these latter anodes and the current supplied to each of them should be adjusted to maintain the desired rate of dissolution of the metals, thus to replenish the metals plated from the bath.

The anodes can be stationary, suitably disposed about the axis of a cylindrical assembly, and agitation can be provided by continuously rotating, in one direction, paddles suspended from a disc between the anode and the surface of the bearing shell, which is immersed in the plating bath. Alternatively, the anodes can be suspended inside of the bearing shell and arranged to rotate. In the latter arrangement, it may be desirable to cyclically reverse the direction of rotation of the anodes to provide a "mixing-agitation" of the solution at the surface of the bearing shell. As a result, fresh solution is supplied to the anode and cathode surfaces during deposition, facilitating control of the physical properties of the plate. Suitable agitation may also be provided by moving the cathode if desired.

Although it is not necessary to provide a diaphragm or anode bags, their use is preferred. Very satisfactory coatings have resulted from enclosing the anodes in bags. When used with rotating anodes, the bags may be suspended so as to rotate with the anodes. For simpler control of the process, it is preferred to use a diaphragm having a cylindrical shape surrounding the anodes. When rotating paddles are used as agitators, they should be separated from the anodes by the diaphragm. The diaphragm serves to contain any particles which may drop

from the anodes, and prevents attachment of the particles to the plated surface with a resulting surface roughness.

Continuous filtration is also desirable and may be accomplished by withdrawing solution from the anode compartment and returning it to the cathode compartment. A filter press can be inserted in the line used for circulating the solution. This press may, or may not, use activated carbon for purification.

The current density will, of course, vary with the composition of the bath, temperature, agitation, etc. However, satisfactory coatings have been deposited with currents varying from 10 to 40 amp. per sq. ft. A periodic current reversal has been found to be beneficial in securing sound deposits, although its use is not essential in this process. The use of such a current tends to eliminate pitting and reduce the amount of roughness and columnar structure. However, the reverse current may also tend to cause brittleness and cracking of the plate.

It is preferable that the steel or other metal surfaces be given a copper strike plate by any of the conventional plating methods, such as a copper cyanide solution. The usual techniques of vapor degreasing, alkaline cleaning, dipping in hydrochloric acid, etc., are used to prepare the surface for the alloy coating. Where small dimensional tolerances are desired, the metal shells can be copper plated and then machined to the proper inside diameter. In such cases a thinner copper-lead alloy plate is desirable as compared to the alloy plate deposited over a copper strike plate. The bearing shell can then be made anodic in the copper-lead alloy plating bath, as a final cleaning operation, before being coated with the alloy.

The following examples will serve to illustrate the invention with greater particularity:

#### Example I

An alloy having a composition of 40 per cent copper and 60 per cent lead was deposited on a steel cathode from the following aqueous bath:

|                                                                                           | G./l. |
|-------------------------------------------------------------------------------------------|-------|
| Potassium pyrophosphate (K <sub>4</sub> P <sub>2</sub> O <sub>7</sub> .3H <sub>2</sub> O) | 100   |
| Potassium cyanide                                                                         | 34    |
| Copper cyanide                                                                            | 22.5  |
| Plumbous chloride                                                                         | 2.7   |

The bath was maintained at 165° F. and operated at a pH of about 8.5. The pH adjustments were made by adding potassium hydroxide (KOH) or hydrochloric acid (HCl). Cast alloy anodes of a composition approximately the same as the alloy coating were used. The current density was 30 amp./sq. ft.

#### Example II

The following aqueous bath was used to form an alloy plating of 40 per cent copper and 60 per cent lead:

|                                     | G./l. |
|-------------------------------------|-------|
| Potassium pyrophosphate             | 100   |
| Potassium cyanide                   | 40    |
| Copper cyanide                      | 22.5  |
| Plumbous chloride                   | 3     |
| Potassium dihydrogen orthophosphate | 20    |

The bath was maintained at a temperature of 130° F., and at a pH value of 8.5. The current density was 10 amp./sq. ft. and the anode and cathode arrangement was similar to that of Example I.

#### Example III

An alloy having a composition of 75 per cent copper and 25 per cent lead was deposited by increasing the bath of Example II to a temperature of 170° F.

#### Example IV

The following aqueous bath was used to deposit an alloy composed of 80 per cent copper and 20 per cent lead:

|                                     | G./l. |
|-------------------------------------|-------|
| Potassium pyrophosphate             | 120   |
| Potassium cyanide                   | 50    |
| Copper cyanide                      | 28    |
| 5 Plumbous chloride                 | 3.5   |
| Potassium dihydrogen orthophosphate | 20    |

The bath temperature was 110° F., and the pH was maintained at about 8.0.

After the copper-lead alloy has been deposited, it is necessary that it be annealed in order to reduce the hardness to a value suitable for bearings. Annealing at temperatures less than 800° F., commonly used for low melting alloys, does not result in sufficient ductility, and causes the formation of two phases from the metastable solid solution of lead and copper. Thus, before the desired softening can be accomplished, lead is sweated out of the alloy and appears on the surface of the bearing and the interface between the alloy and the basis material as globules of pure lead or lead containing a small amount of copper. This physical structure is highly undesirable and detrimental to the performance of the bearing as was noted hereinbefore.

In accordance with the present procedure, exposure to temperatures of about 1000° F. for short period of time in a non-oxidizing atmosphere will soften and anneal the copper-lead alloy plates to a hardness value that is suitable for bearing metals. Induction heating could accomplish this result, but the annealing of large bearing shells having a thin liner would require large and expensive induction heating equipment. Very satisfactory results have been obtained with these alloys by immersion thereof in a fused salt bath, the procedure being the same as disclosed in copending application Serial No. 295,542, filed June 25, 1952.

Although the preceding description of the novel copper-lead alloy coating and the process for depositing it have been described for use in bearing liners, the alloy can be electrodeposited by other techniques and equipment commonly used in the plating industry. For example, a satisfactory copper-lead coating can be formed on a flat panel which is suspended from a moving work bar oscillating back and forth in the plating solution. The plate can also be deposited in a closed circuit in which the solution is circulated by pumps and flowing at a suitable rate in a tube or pipe. The tube or pipe is then coated with the alloy electroplate.

From the foregoing it will be seen that by the present invention copper-lead electrodeposits may be obtained in satisfactory form, and, particularly in the case of bearing linings, such deposits may be suitably obtained in the form of high-copper, low-lead alloys. There has also been disclosed a subsequent annealing process by which the hardness of the alloy plate may be reduced without segregation of the lead in the alloy and without formation of any lead interface layer between the alloy coating and the base material.

Thus, while we have illustrated and described the preferred embodiments of our invention, it is to be understood that these are capable of variation and modification, and we therefore do not wish to be limited to the precise details set forth, but desire to avail ourselves of such changes and alterations as fall within the purview of the following claims.

We claim:

1. A method of electrodepositing on an article arranged as a cathode a copper-lead alloy including the step of passing an electric current through an aqueous bath containing, as the essential ingredients for co-depositing copper and lead on said article, copper cyanide in a concentration of about 22.5 to 28 grams per liter as the source of copper for the alloy, free cyanide to suppress copper ionization, and lead pyrophosphate as the source of lead for the alloy, said lead pyrophosphate being derived from a soluble lead salt in a concentration of about 2.7 to 3.5 grams per liter and alkali metal pyrophosphate

salt in a concentration of about 100 to 120 grams per liter, said bath having a pH of about 8 to maintain lead pyrophosphate in solution.

2. An electrodepositing bath for co-depositing copper and lead as an alloy comprising, as the essential ingredients for co-depositing copper and lead, copper cyanide in a concentration of about 22.5 to 28 grams per liter as the source of copper for the alloy, free cyanide to suppress copper ionization, and lead pyrophosphate as the source of lead for the alloy, said lead pyrophosphate being derived from a soluble lead salt in a concentration of about 2.7 to 3.5 grams per liter and alkali metal pyrophosphate salt in a concentration of about 100 to 120 grams per liter, said bath having a pH of about 8 to maintain lead pyrophosphate in solution.

3. A method of electrodepositing copper-lead alloys containing from about 5 to about 95 per cent lead on an article arranged as a cathode, including the step of passing an electric current through an aqueous bath containing, as the essential ingredients for co-depositing copper and lead on said article, copper cyanide as the source of copper for the alloy, free cyanide to suppress copper ionization, and lead pyrophosphate as the source of lead for the alloy, said lead pyrophosphate being derived from a soluble lead salt and an alkali metal pyrophosphate salt, and said bath having a pH of about 8 to maintain lead pyrophosphate in solution.

4. An electrodepositing bath, containing as the essential ingredients for co-depositing copper and lead as an alloy, copper cyanide as the source of copper for the alloy, free cyanide to suppress copper ionization, and lead pyrophosphate as the source of lead for the alloy, said lead pyrophosphate being derived from a soluble lead salt and alkali metal pyrophosphate, and said bath having a pH of about 8 to maintain lead pyrophosphate in solution.

5. A method of producing a bearing shell lined with a copper-lead bearing alloy comprising the steps of disposing the shell as a cathode to be plated in an aqueous electroplating bath containing as the essential ingredients for co-depositing copper and lead, copper cyanide as the source of copper for the alloy, free cyanide to suppress copper ionization, and lead pyrophosphate derived from a soluble lead salt and alkali metal pyrophosphate as the source of lead for the alloy, said bath having a pH of about 8 to maintain lead pyrophosphate in solution, and after the deposit has been obtained rapidly annealing the lining at a temperature about 800° F. to reduce the lining to bearing softness.

6. A method of producing a bearing shell electrolytically lined with a copper-lead bearing alloy comprising the steps of disposing the shell as a cathode to be plated in an aqueous electroplating bath containing copper cyanide in a concentration of about 22.5 to 28 grams per liter as the source of copper for the alloy, alkali metal cyanide in a concentration of about 34 to about 50 grams

per liter to provide free cyanide to control copper ionization, and lead pyrophosphate as the source of lead for the alloy, said lead pyrophosphate being derived from a soluble lead salt in a concentration of about 2.7 to 3.5 grams per liter and alkali metal pyrophosphate in a concentration of about 100 to 120 grams per liter, said bath having a pH of about 8 to maintain lead pyrophosphate in solution, and after the deposit has been obtained rapidly annealing the lining at a temperature of about 800° F. to reduce the lining to bearing softness.

7. A method of electrodepositing copper-lead alloys on an article to be plated arranged as a cathode including the step of passing an electric current through an aqueous bath containing copper cyanide in a concentration of about 22.5 to 28 grams per liter as the source of copper for the alloy, alkali metal cyanide in a concentration of about 34 to 50 grams per liter to provide free cyanide to control copper ionization, and lead pyrophosphate as the source of lead for the alloy, said lead pyrophosphate being derived from a soluble lead salt in a concentration of about 2.7 to 3.5 grams per liter and alkali metal pyrophosphate in a concentration of about 100 to 120 grams per liter, said bath having a pH of about 8 to maintain lead pyrophosphate in solution.

8. An aqueous electrodepositing bath for depositing a copper-lead alloy on an article to be plated arranged as a cathode and containing copper cyanide in a concentration of about 22.5 to 28 grams per liter as the source of copper for the alloy, alkali metal cyanide in a concentration of about 34 to 50 grams per liter to provide free cyanide to control copper ionization, and lead pyrophosphate as the source of lead for the alloy, said lead pyrophosphate being derived from a soluble lead salt in a concentration of about 2.7 to 3.5 grams per liter and alkali metal pyrophosphate in a concentration of about 100 to 120 grams per liter, said bath having a pH of about 8 to maintain lead pyrophosphate in solution.

#### References Cited in the file of this patent

#### UNITED STATES PATENTS

|           |               |               |
|-----------|---------------|---------------|
| 923,864   | Levy          | June 8, 1909  |
| 1,397,514 | Haines et al. | Nov. 22, 1921 |

#### FOREIGN PATENTS

|         |               |              |
|---------|---------------|--------------|
| 361,892 | France        | Nov. 7, 1906 |
| 1,657   | Great Britain | of 1897      |
| 10,133  | Great Britain | of 1915      |

#### OTHER REFERENCES

Monthly Review, American Electroplaters' Society, vol. 33, 1946, pages 18-23 and 88.  
 Trans. Electrochemical Society, vol. 73, 1938, pages 384 and 406.  
 Treatise on Chemistry, vol. II, 1913, page 899.  
 Trans. Electrochemical Society, vol. 73, 1938, pages 384-394, 405 and 406.